

Patented Nov. 13, 1928.

1,691,654

# UNITED STATES PATENT OFFICE.

ROBERT W. HENRY, OF PORT ARTHUR, TEXAS, AND ELFORD D. STREETER, OF BAYONNE, NEW JERSEY, ASSIGNEES TO GULF REFINING COMPANY, OF PITTSBURGH, PENNSYLVANIA, A CORPORATION OF TEXAS.

## PROCESS OF MAKING THICKENED LUBRICATING OIL.

No Drawing. Application filed March 24, 1926, Serial No. 97,115. Renewed October 3, 1928.

This invention relates to processes of making thickened lubricating oil; and it comprises a method of producing an improved lubricating oil of the type sometimes known as mineral castor oil and consisting of lubricating oil containing a dissolved or dispersed basic aluminum oleate or other basic aluminum soap wherein a sodium soap solution is precipitated by a partially neutralized or 10 basic solution of aluminum sulfate or other aluminum salt; all as more fully hereinafter set forth and as claimed.

In the art what are known as mineral castor oils or castor machine oils are extensively made by thickening mineral lubricating oils by an addition of a certain amount of aluminum oleate. This oleate is ordinarily a trioleate; that is, each atom of aluminum is combined with three oleic acid groups. These 20 trioleate preparations are generally made by direct precipitation of a solution of sodium oleate by an aluminum sulfate solution in the proper proportions. The precipitated aluminum soap so made is separated from the 25 mother liquor, which is a solution of sodium sulfate, washed, dried and added to the mineral oil to be thickened. The oleate goes into solution or dispersion and gives a great increase in viscosity; the result wanted. In the 30 usual types of mineral castor oil however this increase is neither regular nor constant. In adding a given quantity of oleate to a given oil, the exact increase in viscosity is uncertain and the viscosity just after incorporation is 35 by no means what it is after the thickened oil has been allowed to stand for a time and "age". There is always a marked drop in viscosity. In United States Patent 1,550,608 is described a castor oil preparation free of the 40 noted disadvantages; this preparation being made with basic oleates in lieu of the trioleate. Aluminum forms three oleates which may be represented, using the symbol R to represent the oleic acid group, as respectively, the tri- 45 oleate  $AlR_3$ , the dioleate  $Al(OH)R_2$ , and the mono-oleate  $Al(OH)_2R$ . In the stated patent it is pointed out that constant preparations may be obtained by the use of basic aluminum oleates; oleates containing less oleic 50 acid than the trioleate. The patent describes a ratio between R and Al of 1.7:1 or 1.8:1 as being most advantageous.

In the present invention mineral castor oils of this patented type are made but by the use

of a different process. In the patent, the material is made by directly uniting oleic acid and aluminum hydrate in the proper proportions. In the present method basic oleate is made by a precipitation method, using a solution of a soda soap and a solution of aluminum sulfate or chlorid. The soda soap need not be pure sodium oleate; other fatty acids, and particularly unsaturated acids of the oleic type, being equivalent for our purposes to oleic acid. 55

In the present process however in lieu of using sodium oleate and aluminum sulfate in the proper proportions to make trioleate, precipitation of the aluminum sulfate solution is by a mixture of caustic soda and sodium oleate together equivalent to the aluminum salt and in such relative proportions as to give a basic aluminum oleate of the type of that described in the patent. Caustic soda with aluminum sulfate solution gives a precipitate of aluminum hydrate,  $Al(OH)_3$ ; oleate gives aluminum trioleate,  $AlR_3$ ; and a mixture of soda and oleate with aluminum sulfate solution gives intermediate products which are what is here wanted. Any desired 70 ratio of R and OH may be thus obtained. Ordinarily we desire to obtain ratios within the limits prescribed in the stated patent. Our best results have been obtained with ratios between OH and R ranging between  $OH_{1.55}R_{1.45}$  75 and  $OH_{1.45}R_{1.55}$ . The foregoing describes the principle of the present invention but in practice the operation is somewhat more complex. 80

The sodium soap used in the present invention may be made from any of the ordinary soap making oils and by any of the ordinary soap making processes. These oils all contain other fatty acids than oleic acid, but for present purposes as stated, these acids are more or less equivalent to oleic acid. Cottonseed oil and corn oil are satisfactory oils for the present purpose. Commercial oleic acid or red oil, is less satisfactory because of its usual content of iron as an impurity. Rape oil may be used but is not as satisfactory as the other oils. 90 Commercial stearic acid, oleo stearin and coconut oil do not give as good products as cottonseed oil. The particular oily materials used however are not as important as the chemical and physical control of the operation 100 as hereinafter set forth.

In a practical embodiment of the present invention a fatty oil is saponified with the

calculated quantity of caustic soda to produce a neutral soap; this being done by any of the ordinary soap making processes. There results a solution containing neutral soda salt of oleic and of the other acids contained in the oil and also containing more or less glycerin. A basic solution of an aluminum salt is prepared by adding caustic soda solution to a solution of aluminum sulfate or 5 chlorid. The concentration of the aluminum salt solution may be 0.5 to 1 pound per gallon; the caustic soda solution may be 5° to 10° Baumé. Basic aluminum sulfate solutions are suitable for preparing aluminum soaps of 10 15 a composition approaching the dioleate; while basic aluminum chlorid solutions are more suitable for preparing the lower ratio soaps; i. e. those whose compositions approach  $AlR_{1.5}(OH)_{1.5}$ . In either case, it is 20 advantageous to add some protective agent such as citric acid or a citrate, tartaric acid or a tartrate, etc. to prevent precipitation of alumina. About 0.1 per cent of disodium citrate in the solution of the aluminum salt 25 will suffice to prevent precipitation of alumina. The neutral soda soap solution is emulsified with a body of lubricating oil to form a pulp, the emulsion is heated to boiling, and the basic aluminum salt solution is added 30 to it. To prepare a soap of the composition  $AlR_{1.5}(OH)_{1.5}$ , the amount of caustic soda added to aluminum chlorid solution is enough to give the ratio  $2AlCl_3:3NaOH$ , and the 35 amount of this basic solution added to the soda soap solution is slightly in excess of enough to give the ratio



This leaves the liquor slightly acid to the 40 usual indicators. The amount of lubricating oil added may be from 1 to 2 times the volume of the fatty oil originally used in making the soap. Within limits, the slower the addition of the aluminum salt solution the better. 45 With a charge of ordinary size, it is recommended that the addition be spread over a period of about 2 hours. It makes a better preparation to continue boiling and stirring for about an hour after the addition of the 50 aluminum salt is completed. At this point, the reaction of the solution in contact with the pulp should be slightly acid;  $P_H$  4.5 is advantageous. Besides the solution of aluminum soap in oil, the batch at this stage contains 55 a water solution of sodium sulfate which must be removed. This is accomplished by washing the pulpy mass with boiling water for about 30 minutes, removing the water, and digesting with a fresh charge of boiling 60 water, and so on, until the separated water shows substantial freedom from sodium sulfate. Three or four washings will usually suffice. The washed material is then dried. This may be accomplished by heating and stirring in an iron kettle. Very careful con-

trol of the drying operation is necessary to produce the best products. Complete dehydration gives a yield of viscosity no higher than the mineral oil, while insufficient drying tends to cause a separation of the colloidal suspension wanted. Between these extremes lies the article desired; a very viscous preparation. This correct point is best determined by the appearance of the material, and may be thus attained by one experienced 70 in the art. Finally, the pulp is diluted by stirring in mineral lubricating oil until the viscosity of the desired commercial grade of castor machine oil is attained.

While we have described a method of making a basic oleate wherein caustic soda is added to aluminum salt solution (the presence of a protective agent such as disodium citrate being advantageous but not necessary) and the mixture used in precipitating a sodium soap solution, similar results may be obtained by adding the caustic soda to the sodium soap solution and precipitating by means of neutral aluminum salt solution. The process so conducted is not quite as advantageous for 80 obtaining the lower ratio soaps, as working in the way described. For making the di-soap, however, working in this way is simpler and less expensive than the method described, in that the basic alum solution need not be made up separately from the sodium soap solution and no protective agent is required. 85

In this second embodiment of the present invention, a fatty oil is saponified with the calculated amount of caustic soda by any of the ordinary soap making processes. A solution of this soap is emulsified with a body of lubricating oil and to this emulsion is added further caustic soda. The amount of mineral oil used in pulping the mixture may 100 be 1 to 2 times the volume of the fatty oil originally used. The amount of added alkali is about enough to give a ratio of  $2NaR:NaOH$ . The alkaline mixture is heated to boiling and aluminum sulfate (or chlorid) solution is added slowly. The amount of alum added is enough to give the ratio  $Al_2(SO_4)_3:NaR:2NaOH$ . The concentration of the alum solution may be 0.5 to 1 pound per gallon. The addition of 105 alum solution should be spread over about 2 hours, and the boiling and stirring should be continued for about an hour thereafter. After the addition, the reaction of the solution in contact with the pulp should be slightly acid;  $P_H$  4.5 is advantageous. The pulp is washed, dried and diluted with mineral oil as described above. By this method a di-soap castor is obtained.

Potash soaps may be used in lieu of soda soaps; and potash in lieu of soda; but such substitution offers no particular advantage and adds to the cost.

The presence of lubricating oil during the manufacture of the basic aluminum oleates 130

while not absolutely necessary is convenient and advantageous. Where it is used it remains with the oleate and forms part of the final thickened lubricating oil or mineral 5 castor oil. The pulp containing the oil is simply diluted with enough more lubricating oil to give the viscosity wanted.

What we claim is:—

1. In the production of mineral castor oil 10 of a constant viscosity and containing basic aluminum oleates, the process which comprises preparing an aqueous solution of soap, preparing a solution of an aluminum salt, and intermixing the two solutions in the 15 presence of alkali, thereby precipitating a basic aluminum soap, and admixing the aluminum soap with mineral oil.

2. In the production of mineral castor oil of constant viscosity and containing basic 20 aluminum oleates, the process which comprises preparing an aqueous solution of soap, and adding a solution of an aluminum salt, in the presence of alkali, thereby precipitating a basic aluminum soap, the amount of 25 aluminum salt so added being sufficient to render the resulting liquor slightly acid.

3. In the production of mineral castor oil of constant viscosity and containing basic aluminum oleates, the process which comprises preparing an aqueous solution of soap, preparing a solution of an aluminum salt, intermixing the two solutions in the presence 30 of alkali added thereto, the quantities of reacting materials being such as to effect the precipitation from the mixture of solutions 35 of an aluminum soap containing less fatty acid than that corresponding to a tri-acid soap, and to render the resulting liquor slightly acid.

4. In the manufacture of mineral castor

oil of constant viscosity and containing basic aluminum oleates, the process which comprises saponifying an oil with the necessary amount of alkali solution to give a neutral soap solution, emulsifying such solution with lubricating oil, precipitating a basic aluminum oleate by adding a solution of aluminum salt made basic by addition of alkali, washing the basic aluminum oleate with hot water to free it of salts, drying, and adding 5 enough mineral oil to produce a mineral castor oil of the desired viscosity.

5. In the manufacture of mineral castor oil of constant viscosity and containing basic aluminum oleates, the process which comprises preparing an aqueous soap solution, and emulsifying lubricating oil therein; separately preparing a basic aluminum salt solution by adding alkali to a solution of an aluminum salt in the presence of a protective 55 agent, such as sodium citrate, in quantity sufficient to prevent the precipitation of aluminum hydroxide; mixing the two solutions in proportions such as to precipitate the water soluble soap in the form of a pulp of basic 60 aluminum soap, washing the pulp so formed with hot water to free it of salts, drying, and adding enough mineral oil to produce a mineral castor oil of the desired viscosity.

In testimony whereof we have hereunto 70 affixed our signatures at the places and on the dates indicated.

Signed at Port Arthur, in the county of Jefferson and State of Texas, this 18th day of March, 1926.

ROBERT W. HENRY.

Signed at Bayonne, in the county of Hudson and State of New Jersey, this 22nd day of March, 1926.

ELFORD D. STREETER.